

Oct. 13, 1942.

C. D. COXE

2,298,348

FORMATION OF METAL SHAPES

Filed May 11, 1940

4 Sheets-Sheet 1

Fig. 1



Fig. 2



Fig. 3



Fig. 4



Fig. 5



INVENTOR  
Charles D. Coxe  
BY  
D. Verner Smythe  
ATTORNEYS

Oct. 13, 1942.

C. D. COXE

2,298,348

FORMATION OF METAL SHAPES

Filed May 11, 1940

4 Sheets-Sheet 2



INVENTOR  
Charles D. Coxe  
BY *John C. Coxe*  
D. Under & Son, Inc.  
ATTORNEYS

Oct. 13, 1942.

C. D. COXE

**2,298,348**

## FORMATION OF METAL SHAPES

Filed May 11, 1940

4 Sheets-Sheet 3



INVENTOR  
Charles D. Coxe  
BY ~~James~~ and  
D. D. Dwyer, Esq., the  
ATTORNEYS

Oct. 13, 1942.

**C. D. COXE**

**2,298,348**

## FORMATION OF METAL SHAPES

Filed May 11, 1940

4 Sheets-Sheet 4

Fig. 17



INVENTOR  
Charles D. Cox  
BY ~~attorneys~~  
D. Lathrop & Co.,  
ATTORNEYS

## UNITED STATES PATENT OFFICE

2,298,348

## FORMATION OF METAL SHAPES

Charles D. Coxe, Bridgeport, Conn., assignor to  
Remington Arms Company, Inc., a corporation  
of Delaware

Application May 11, 1940, Serial No. 334,537

12 Claims. (Cl. 22—57.2)

The invention relates to a method and apparatus for the making of metallic shapes directly from a molten metal, and is particularly adapted for the production of such things as metallic sheets which are relatively thin, and for the production of spherical objects such as balls or shot. The making of sheets has been previously accomplished in various manners.

In the manufacture of a metallic sheet or strip, one method commonly used is that of casting the metal into a relatively thick ingot and then successively rolling the ingot to the desired thickness, this being done in a plurality of rolling operations requiring heavy and large machinery. It is also necessary to reheat during the reduction process, and much labor is required to operate the equipment. In the rolling and forging operation in the reduction of the ingot, there is considerable loss due to scaling and waste in the ingot itself.

Another method of producing strip metal or sheet is by the pouring of the molten metal directly between two rotating rolls, such as in Hazelett, No. 2,058,447, the rolls being cooled and rotated as the metal is poured therebetween, these rolls generally being horizontal. Another process shown in the patent to Coxe, No. 2,183,010, uses four adjacent vertical rolls. In both of these types of casting directly onto the rolls, the surface metal is solidified as contact is made with the rolls. It is evident that in such a process, much difficulty will result from unevenness in the rolls, the tendency of the metal to cling to the roll surfaces, and rapid deterioration of the rolls due to the hot metal impinging thereon. All these matters tend to produce defective sheets and require expensive equipment.

The making of round or spherical objects also heretofore has required expensive machinery or the use of high towers for the dropping of the metal in its molten form, which will assume a spherical form before it reaches the bottom of the tower, such as in the conventional shot tower.

In the invention disclosed herein, a molten metal bath is provided, having a lower melting point than the metal to be shaped and a boiling point which is higher than the freezing point of the metal to be shaped. The metal of the molten bath and the metal to be shaped must be immiscible, or substantially immiscible, both in the liquid and solid state, and preferably have a different specific gravity so that they may be properly separated from each other. By im-

miscible, it is not meant that the metals absolutely are not immiscible but that the immiscibility is such that they may be readily separated. The metal being shaped should also have sufficient hot tenacity to hold itself together as it is being withdrawn.

The other objects of the invention will appear from the detailed description and drawings following, which give several forms of the invention and are merely for the purpose of illustration.

In the drawings:

Fig. 1 is a diagrammatic side elevation of one type of apparatus, with a portion cut away, that may be used to produce metal sheets.

Fig. 2 is a detailed side elevation, partially in section, of an apparatus similar to that of Fig. 1, but not having the cleaning rolls.

Fig. 3 is a plan view of Fig. 2.

Fig. 4 is a cross sectional view of Fig. 2 taken from the line 4—4 of Fig. 2.

Fig. 5 is a fragmentary cross sectional elevation of a modification of the molten metal bed of the apparatus shown in Fig. 1.

Fig. 6 is a fragmentary elevation of a modified apparatus for forming sheets.

Fig. 7 is a sectional elevation taken at line 7—7 of Fig. 6.

Fig. 8 is a plan view of the apparatus shown in Fig. 6.

Fig. 9 is a fragmentary side elevation of a modification of the apparatus shown in Fig. 6.

Fig. 10 is a sectional side elevation of a modification of an apparatus for forming sheets.

Fig. 11 is a sectional plan view of the apparatus shown, taken on line 11—11 of Fig. 10.

Fig. 12 is a diagrammatic view of a modification of an apparatus for making sheets, wherein the specific gravity of the metal being shaped is greater than that of the bath.

Fig. 13 is a cross sectional side elevation of an apparatus for making individual metal shapes, such as round balls or shot.

Fig. 14 is a sectional view taken at the line 14—14 of Fig. 13.

Fig. 15 is a diagrammatic sectional view of one form of nozzle and closure therefor, shown in Fig. 13.

Fig. 16 is a fragmentary view of a cooling roller that can be used in conjunction with the forming of sheets.

Fig. 17 is a cross sectional side elevation of an apparatus for making individual metal shapes, such as round balls or shot.

In general, as has been stated, the metal of the

molten bath is one having a lower melting point and a higher boiling point than the freezing point of the metal which is to be shaped, and the specific gravity of the molten bath may be either greater or less than the specific gravity of the metal to be shaped, depending upon the mode in which the invention is carried out, as will become apparent in the description of the invention which follows.

For example, when a sheet is to be cast or formed on the top of a molten bath, it is evident that the molten bath must have a higher specific gravity so that it will stay at the bottom and the metal which is to be shaped will lie on top thereof. In the making of such a metal sheet, when the molten metal to be shaped is poured upon the surface of the molten bath, it is necessary, except in a device such as shown in Figs. 1 and 2, that a strip of the metal similar to the molten metal to be shaped be placed on the top of the molten bath so as to contact the molten metal to be shaped as it is poured onto the bath. The metal will start to freeze to the solid piece, and the strip may be moved over the surface of the molten bath, causing more of the metal to freeze thereto, and thus be drawn along the surface of the bath and then removed from the bath continuously or in the length desired. It is also evident that the metal to be shaped may be one that has a greater specific gravity than the molten bath, in which case the molten bath will lie on top of the molten metal to be shaped and the freezing will take place at the interface of the two metals, which, in this case, will be the upper surface of the metal strip. It is also evident that in many cases the exterior of the metal strip will become frozen and the interior might still be in a molten or plastic form, as it is first formed, but will become completely solid very shortly after the initial forming or after its removal from the molten bath.

In the formation of spherical objects, such as shot, a molten bath having a greater specific gravity than the metal to be shaped may be used, and the molten metal to be shaped introduced at the bottom of the bath. When this is done, a nozzle may be so arranged that the molten metal to be shaped will flow upwardly through the bath in particles or globules which will become spherical due to the surface tension of the metal and will freeze at the interface of the two metals so that by the time it reaches the top of the molten bath the metal object will have obtained its spherical form. It is also evident that this process may be reversed and the specific gravity of the molten bath be less than that of the metal to be shaped, and the molten metal allowed to drop into the molten bath, and the spherical shapes removed from the bottom of the bath. The temperature of the bath and metal must be so regulated as to allow the proper shaping of the globules as they pass through the bath.

As an example of two metals that may be used, lead having a melting point of 621° F., a boiling point higher than 2800° F., and a specific gravity of 11.34 may be used as the molten bath; and aluminum having a melting point of about 1220° F. and a specific gravity of 2.7 may be used as the metal to be shaped. In this case, if sheets or flat objects are being made, the aluminum will float on a surface of the molten metal and may be withdrawn therefrom in the manner about to be described. If aluminum shot or spherical objects are to be made, the metal may be introduced at the bottom of the molten lead bath, and the

aluminum will travel upwardly through the bath, attaining a spherical form by the time they reach the top of the bath, it being evident, of course, that the depth of the bath must be made such and the temperatures kept at such a point that the balls will attain their spherical form by the time they reach the surface.

Steel or iron having a melting point of about 1535° C. may be used in place of aluminum. As 10 other examples, silver may be used as the molten bath for the shaping of chromium and nickel, silver having a lower melting point than chromium and nickel and having a higher specific gravity. Bismuth or cadmium may also be used as the 15 molten bath for the formation of the aluminum shapes.

If, for example, aluminum be maintained at a temperature of about 690° C. and most of the 20 lead kept at a temperature of about 400° C., the aluminum will freeze at the interface of the two metals. The resultant layer of aluminum can be removed, making room at the interface for another portion of the aluminum to freeze; and the frozen aluminum may be removed continuously and thereby form a continuous strip or a strip of the length desired.

The invention will be first described in conjunction with its application to the manufacture of such things as metal sheets, and particularly to the continuous production of metal sheets which are comparatively thin, relative to their width.

Referring particularly to Fig. 1, the molten metal to be shaped is poured into the receptacle 28 having a spout or outlet 21. A molten metal bath 22 is held in the container 23. In the modification shown in Fig. 2, the molten metal bath is a metal that has a higher specific gravity than the metal being shaped and a lower melting point. The molten bath as previously described must also have a higher boiling point than the melting point of the metal to be shaped. As an example of the means that might be employed to withdraw the metal as it is formed over the top of the molten bath, the two endless chains or engaging means 24 may be suitably driven through gears 25 and shaft 26 from some suitable source of power, the chains being advanced in the direction shown by the arrows in Fig. 3. As the strip of metal reaches the end of the container 23 (Fig. 2), it may pass through a slot 21 and be gripped by the rollers 28 and carried to its point of storage, or where it is to be further operated upon. The rolls 28 may also be so designed as to cause a shaping action to be exerted upon the sheet at this point. As the molten metal flowing from the container 23 comes into contact with the surface of the molten bath 22, freezing will occur at the interface of the metals, the portion away from the interface still remaining liquid, depending upon the relative difference of temperatures between the baths and thickness of the sheet to be formed and other factors. The sheet 29 passes into engagement with the endless chains 24 and has its width limited thereby, and as it continues in its passage through the container 23 it will solidify substantially throughout its thickness. As will be explained later, the rate of solidification affects the type of surface obtained upon the sheet. In order to prevent oxidation of the metal sheet being formed and of the bath, an inert atmosphere may be superimposed over the sheet and bath by means of the cover 30 in any of the conventional and usual manners; for example, the inert atmosphere may

be supplied through the pipe 31 (Fig. 1) and the exit slit, such as at 32 or 27 (Fig. 2), may be made to retain the inert atmosphere within the container 30. Because the sheet being formed is of necessity at a higher temperature than the bath, it is evident that the molten bath will absorb heat from the metal being shaped, and therefore the bath must be cooled or so designed that the proper temperature differential will be maintained. This may be done in many ways, as an example thereof, the molten bath material may be drawn into the pipe 33 (Fig. 1) and passed through a suitable cooler 34. A pump 35 may be employed to return the molten bath material to the container 23 at a temperature such that the metal sheet will properly form on the metal bath at its point of impingement therewith. Cleaning wheels, such as shown diagrammatically at 36 (Fig. 1), may be employed upon either side of the strip to clean the molten lead therefrom and any scale that may have formed before it passes between the pinch rolls 37 to the point of storage. If desired, an air blast (not shown) may be directed against the bottom of the sheet before it leaves 30 so as to remove the molten bath metal that might be clinging thereto. It is to be noted that Fig. 1 differs from Fig. 2 in that Fig. 1 has the cleaning rolls 36.

In the formation of the sheet, several means may be employed to obtain a top surface which will be either absolutely smooth or may be easily rolled to a smooth surface. If the rate of cooling of the strip is rapid, but not quite rapid enough, pits will be formed in the sheet similar to the sink holes in ingots. A dendritic-like structure may also form on the surface when complete cooling takes place on the bottom, so that the top surface is the last to freeze. One means of avoiding this is to provide a cooled roller, such as shown diagrammatically in Fig. 16 at 38, touching the top surface of the metal sheet being formed, which will cause the upper surface to freeze smoothly, the lower surface only having been frozen at the interface of the two metals. If there is any molten metal still left, it will be at the interior of the sheet, and no pits will be formed in the surface of the sheet. It is also possible to similarly cool the upper surface of the metal by passing the inert atmosphere through a cooler and directing it over the surface of the metal or by other similar means. A smooth surface may also be obtained by providing a heater, such as gas flames or an electric induction heater, over the metal strip after it has been formed, so as to liquify a layer on the upper surface which may then cool uniformly to present a smooth surface.

In Fig. 5 is shown an alternative form of molten bath and cooling means therefor, which may be used instead of that shown in Figs. 1 to 4. The metal sheet 39 is supported by the relatively thin molten bath 40, which in turn is supported upon a bed 41 having cooling holes 42 running therethrough. A suitable means may be used to force a cooling medium through holes 42.

The metal sheet may also be formed, particularly when it is thin, by means of the apparatus shown in Figs. 6 to 8. In this form, the receptacle for the molten metal to be shaped is at 43 and it has an opening 44, allowing the molten metal to flow out upon the surface of the molten bath. This molten bath may take the form shown in Fig. 1 or Fig. 5. Metal is poured into the receptacle and allowed to flow onto the molten bath, and drawn along the bath by any suitable

means. The rollers 45 may be employed to do this and to cause the edges of the strip to be of uniform width.

The thickness of the sheet can be regulated by the feeding slot and by the rate at which the forming strip is withdrawn.

In the event that it is desired to place a second layer upon the first layer, it is also possible to provide a second container, such as shown at 45 of Fig. 9, and thereby form a second layer upon the first layer that has already been formed. It is evident that a different metal may be used for this purpose or the same metal. Such a method might have application in the formation of bimetallic strips for use in thermostatic devices.

Figs. 10 and 11 show still another modification of the apparatus just described which can be used for making a metal sheet directly from the molten metal wherein the sheet being formed 20 has a higher melting point and a lower specific gravity than the molten bath. A burner 46 may be employed to heat a combustion chamber 47 under the container 48, which will serve to keep the molten bath, such as lead in 49, at the proper 25 temperature. The metal to be formed is introduced in the molten form through the opening 50 and will collect in the top of the chamber 51 as at 52. In order to insure that this remains in a molten state, a fuel and air supply may be provided at 53 to heat the metal 52. A circulating and cooling means for the lead is provided, having an intake 54 withdrawing the lead and passing it through a cooler from pipe 55 and returning it through pipe 56 to the nozzle 57. Nozzle 57 is 30 so arranged as to direct the cooled lead against the surface of the metal sheet being formed at the junction of the molten bath 49 and the metal to be shaped 52. It is necessary in starting the operation to introduce a small piece of the sheet 35 already formed, to which the molten metal will cling and which can be withdrawn through the opening 58, between the rolls 59, and out of the bath through opening 60 and between the rolls 61. An inert atmosphere may be introduced into 40 the container 62 through pipe 63. Suitable means may be employed to cool the portion of the bath near the sheet being moved therethrough by the pipe 64, withdrawing the molten metal and passing it through a suitable cooling 45 means, and returning the molten metal to this portion of the bath by the pipe 65 which is directly over the roll 59, serving to cool the roll and to further cool the metal strip.

In the event that the metal to be shaped has a 55 higher specific gravity than that of the molten bath, the apparatus diagrammatically shown in Fig. 12 may be employed. In this case the molten metal to be shaped is introduced through means 66 into the portion 67 having a separating wall 68. The molten metal 69 is on top of the metal of the sheet being formed, and a strip is started at the interface of these surfaces and led between the rolls 70, and may then be withdrawn. The metal will freeze at the interface of these 60 metals and may thus be withdrawn in a manner similar to that just described.

By the invention described herein, metal objects may also be formed, such as spherical or similar objects, by the apparatus shown in Figs. 13 and 14. The metal to be shaped may be poured into the tower 71 through a spout 72. The molten bath to be used in the forming of the objects is located at 73, wherein there is a metal having a higher specific gravity and lower melting point than the metal to be shaped. A nozzle may be

provided at 74 through which the metal passing down the tower 71 through passages 75 and 76 may be introduced at the bottom of the molten bath 77. It is to be understood that there may be more than one nozzle and that the nozzle may take various forms, sizes and shapes, in dependence upon the object that is to be produced. In the specific form shown, there is a graphite plate 78, which may be heated by suitable electric means which will keep the nozzle clear and prevent the freezing of metal at this point. To start the device, a rivet 79 or similar article may be placed within the hole, and when a sufficient head of metal has been placed in the tower 71, the rivet 79 will be forced from the hole and will allow the passage of the metal upwardly through the molten bath 77. It is evident that many other means may be employed to control this opening, and that this is merely an example of a means that might be employed. The metal objects will cool at the top of the bath 77, such as at 80, and may be removed through the opening 81 in any suitable manner.

The metal objects thus formed will be spherically shaped, and such things as metal shot may be so made.

It is also evident that the specific gravities of the metal to be shaped and the molten bath may be reversed and the shot dropped through the bath. Suitable apparatus for carrying out this idea is shown in Fig. 17.

The molten bath 77 may have suitable insulating means such as at 82 to keep the bath at a suitable temperature to allow the desired spherical shape to be attained.

By the invention disclosed herein, a molten bath having a melting point lower than that of the metal to be shaped and immiscible therewith may be employed in the shaping of metal objects directly from molten metal, thus eliminating much of the waste and heavy machinery used in previous methods. As this is the first time that a satisfactory method and apparatus have been developed for such a purpose, the invention is not limited to the details disclosed herein, but is to be construed as broadly covering all equivalent devices and processes falling within the scope of the appended claims.

What is claimed is:

1. In the continuous manufacture of metal sheets directly from molten metal, the process comprising the steps of providing a bath of molten metal substantially immiscible with and having a lower melting point and different specific gravity than the metal to be formed into sheets; spreading a sheet of the molten metal into contact with the molten bath whereby a sheet of the molten metal to be shaped will freeze at the interface of the metals; and then continuously removing the frozen metal sheet from the bath.

2. In an apparatus for shaping metallic objects directly from molten metal, the combination comprising means to supply the molten metal to be shaped; a substantially stationary molten metal bath container to form a planar surface molten metal bath; a molten metal in said container, said second molten metal being substantially immiscible with and having a lower melting point than the first mentioned metal; and means for effecting controlled delivery of the metal to be shaped directly to a surface of the metal of said bath.

3. In an apparatus for shaping metallic objects directly from molten metal, the combina-

tion comprising means to supply the molten metal to be shaped; a substantially stationary molten metal bath container to form a planar surface molten metal bath; a molten metal bath in said container, said second molten metal being substantially immiscible with and having a lower melting point and a higher specific gravity than the first mentioned metal; and means for effecting controlled delivery of the metal to be shaped directly to a surface of the metal of said bath.

4. In an apparatus for shaping composite metallic sheets directly from molten metal, the combination comprising a container for a substantially planar surface molten metal bath; a molten metal bath in said container, said molten metal of the bath being substantially immiscible with and having a lower melting point than the metal of the sheet to be formed directly thereon; means for effecting controlled delivery of a molten metal directly to a surface of the metal of the bath so that freezing will occur at the interface of the metals; and means for effecting a controlled delivery of a second stream of molten metal onto the at least partially frozen first molten metal.

5. In an apparatus for shaping metallic objects directly from molten metal, the combination comprising means to supply the molten metal to be shaped; a substantially stationary molten metal bath container, a molten metal in said container, said last mentioned molten metal being substantially immiscible with and having a lower melting point than the first mentioned metal; means for effecting controlled delivery of the metal to be shaped directly to a surface of the metal of said bath; and means for controlling the temperature of the portion of the second molten metal adjacent the metal to be shaped.

6. In an apparatus for producing metal shapes directly from a molten metal, the combination comprising a container for the metal to be shaped; a stationary container; a molten metal bath in said stationary container, the metal of said bath being substantially immiscible with and having a lower melting point than the metal to be shaped; means for effecting controlled delivery of the metal to be shaped directly to a surface of the metal of said bath so that freezing will occur at the interface; a supporting body associated with said bath metal container having temperature controlling passages therethrough; and means to remove the formed metal shapes from the surface of said bath.

7. In an apparatus for forming metal sheets directly from molten metal, the combination comprising: a molten metal bath container, a molten metal in said container, said last mentioned molten metal being substantially immiscible with and having a lower melting point than the first mentioned metal; means to feed a sheet of the molten metal to be shaped into contact with the molten metal bath so that freezing will occur at the interface of the two metals; means to move the at least partially frozen sheet along the surface of the molten metal bath; and means to remove the at least partially frozen sheet from the molten metal bath.

8. In an apparatus for forming metal sheets directly from molten metal, the combination comprising: a molten metal bath container, a molten metal in said container, said last men-

tioned molten metal being substantially immiscible with and having a lower melting point and higher specific gravity than the first mentioned metal; means to feed the molten metal to be shaped onto the surface of the molten metal bath so that freezing will occur at the interface of the two metals; means to engage the edges of the sheet being formed to move the sheet along the surface of the molten metal bath; and means to remove the at least partially frozen sheet from the molten metal bath.

9. In an apparatus for forming metal sheets directly from molten metal, the combination comprising: a molten metal bath container, a molten metal in said container, said last mentioned molten metal being substantially immiscible with and having a lower melting point and higher specific gravity than the first mentioned metal; means to feed the molten metal to be shaped onto the surface of the molten metal bath so that freezing will occur at the interface of the two metals; means including two endless engaging means for engaging the opposite edges of the sheet being formed so as to move the sheet along the surface of the molten metal bath; and means to remove the at least partially frozen sheet from the molten metal bath.

10. In an apparatus for shaping metal sheets directly from a molten metal, the combination comprising: a molten metal bath container, a molten metal bath being substantially immiscible with and having a lower melting point than the first mentioned metal; means to feed the molten metal to be shaped into contact with the molten metal bath so that freezing will occur at the interface of the two metals; means including two endless engaging means for engaging the opposite edges of the sheet being formed so as to move the sheet along the surface of the molten metal bath; and means to remove the at least partially frozen sheet from the molten metal bath.

11. In an apparatus for shaping metal sheets directly from molten metal, the combination comprising: a molten metal bath container, a molten metal in said container, said last mentioned molten metal being substantially immiscible with and having a lower melting point than the first mentioned metal; means to feed a sheet of the metal to be shaped into contact with the molten metal bath so that freezing will occur at the interface of the two metals; means to cool the face of the sheet opposite to that first frozen; and means to remove the at least partially frozen sheet from the molten metal bath.

12. In an apparatus for shaping metal sheets directly from molten metal, the combination comprising: a molten metal bath container, a molten metal in said container, said last mentioned molten metal being substantially immiscible with and having a lower melting point than the first mentioned metal; means to feed the metal to be shaped into contact with the molten metal bath so that freezing will occur at the interface of the two metals; means to cool the face opposite to that first frozen comprising a cooled roller to contact the face of the sheet opposite to that in contact with the molten metal bath; and means to remove the at least partially frozen sheet from the molten metal bath.

13. In an apparatus for shaping metal sheets directly from molten metal, the combination comprising: a molten metal bath container, a molten metal in said container, said last mentioned molten metal being substantially immiscible with and having a lower melting point than the first mentioned metal; means to feed the metal to be shaped into contact with the molten metal bath so that freezing will occur at the interface of the two metals; means to cool the face opposite to that first frozen comprising a cooled roller to contact the face of the sheet opposite to that in contact with the molten metal bath; and means to remove the at least partially frozen sheet from the molten metal bath.

CHARLES D. COXE,